

## UNITED STATES PATENT OFFICE.

HAROLD H. OSBORNE, OF NIAGARA FALLS, NEW YORK, ASSIGNOR TO AMERICAN MAGNESIUM CORPORATION, OF NIAGARA FALLS, NEW YORK, A CORPORATION OF NEW YORK.

## PROTECTING MOLTEN MAGNESIUM.

No Drawing.

Application filed October 27, 1922. Serial No. 597,380.

My invention relates to a method of protecting molten magnesium from the air to avoid burning of the metal. Magnesium is exceedingly active chemically and at slightly above its melting point, 651 degrees C., will combine with both oxygen and nitrogen of the air. In melting and casting magnesium and high magnesium alloys, it is necessary to provide some means to protect the metal from burning, otherwise the cast metal will have magnesium compounds occluded in it, which cause defects and weaknesses in the castings. In fact, failure to protect the metal from burning may result in the complete consumption of the magnesium before it can be cast.

For attaining the desired end, I have discovered that if a small quantity of glycerine, preferably anhydrous, is brought into contact with the molten metal in a closed receptacle, that burning of the magnesium is obviated and that no deleterious products are formed resulting from decomposition of the glycerine so that the finished castings are free from imperfections with a consequent improvement in their physical properties.

The glycerine may be added at the beginning of the melt and it may be added from time to time as the melting proceeds. In practice, however, there is a cover on the pot and while it is not gas tight, it might be called circulation tight, that is to say, it prevents the ready escape of the vapors which may be formed by the breaking down of the liquid or vaporized glycerine.

In starting a melt, the charge of magnesium containing metal having been placed in the furnace, a few cubic centimeters of as nearly anhydrous glycerine as possible are added, all openings are covered with rather close fitting covers, and the heat is turned on. During the pouring or tapping, and whenever it is necessary to expose the interior of the pot to the open air, a few additional drops of glycerine are added so as to always keep the pot filled with glycerine vapor and to exclude the air.

The theory upon which glycerine acts to prevent oxidation of the molten metal in a closed receptacle may be explained in part as follows:

Glycerine boils at approximately 290 degrees C. while magnesium melts at 651 de-

grees C. Accordingly, when the metal is molten, the glycerine or product thereof will be in the form of a vapor and is effective because it excludes the air and at the same time, it does not quickly react with the molten magnesium. The specific gravity of the vapor of glycerine at the melting point of the metal is comparatively high and for that reason it does not escape easily from a fairly well closed up vessel. When a small quantity of glycerine is brought into contact with the molten metal, the volume of the vapor is many times the volume of the initial liquid material. The glycerine vapor originates in the lower portion of the gas space which is over the metal and the tendency accordingly is to gradually but continuously force out the air through a purposely left open vent in the cover. It is possible, therefore, that the space above the metal is entirely filled with glycerine vapor and inasmuch as glycerine does not seem to react at fairly low temperatures with magnesium, the magnesium does not undergo any appreciable loss.

This is probably the condition during the early stages of melting when the temperature is still fairly low. As the temperature rises, the glycerine vapor begins to form other compounds which also afford protection to the molten metal but not combining with it. Ultimately there is, of course, a complete decomposition of the glycerine or at least an escape of it from the pot which is the practical reason why a small quantity is intermittently added during the melting operation.

As the temperature of the metal approaches its melting point, glycerine being an organic substance is fairly easily changed into other compounds when its vapor is brought to such an elevated temperature. The strong reducing action of the magnesium probably promotes the decomposition.

Glycerine is a trihydric alcohol having the formula  $C_3H_5(OH)_3$ . When glycerine vapor is heated above its boiling point it may form either decomposition products, which are of lower molecular weight or polymerized products which are of higher molecular weight. It is believed, therefore, that these products are as effective in protecting the magnesium as is the glycerine itself, except as the lighter weight molecules more easily

escape from the closed pot. Of the polymerized products, diglycerine has been found to be as effective as is the monoglycerine.

In my U. S. Patent #1,533,892 I have described and claimed the use of glycerine in sand molds for the purpose of preventing the burning of magnesium. In this present application therefore I do not claim the use of the glycerine or equivalent materials in the mold material but only the addition of such substances to such surface or surfaces of molten magnesium or its alloys as would otherwise be freely exposed to the air, such as surfaces in the melting crucible or pouring stream; and as the continuation of this stream surface, the surfaces of the molten metal in the openings of the mold where it is freely exposed to the air.

I claim:

- 20 1. The method of protecting molten magnesium and magnesium alloys comprising bringing in contact with the molten metal, products resulting from the heating of glycerine above the melting point of said metal.
- 25 2. The method of protecting molten magnesium and magnesium alloys comprising treating the molten metal in a closed receptacle from time to time with a relatively small quantity of glycerine.
- 30 3. The method of protecting molten magnesium comprising treating the molten magnesium in a closed receptacle with a relatively small quantity of glycerine and providing a vent in the said receptacle to permit escape of the displaced gases.
- 35 4. A method of protecting molten mag-

nesium and magnesium alloys against burning during melting and pouring, comprising bringing in contact with the surface of the metal in a receptacle, a material having a boiling point which is relatively high but lower than the melting point of the metal, the said material in a gaseous condition serving to prevent burning of the metal, without itself reacting excessively with the molten metal.

5. A method of protecting molten magnesium and magnesium alloys against burning during melting and pouring, comprising bringing in contact with the surface of the metal in a closed receptacle, a material having a boiling point which is relatively high but lower than the melting point of the metal, the said material in a gaseous condition serving to prevent burning of the metal, without itself reacting excessively with the molten metal, the specific gravity of the said material in a gaseous condition being relatively high, whereby it does not readily escape from the closed receptacle.

6. Method of protecting molten magnesium and magnesium alloys against burning at surfaces freely exposed to the air, comprising bringing in contact with such surface of the molten metal a material having a boiling point between about 290° C. and 650° C., which will react only slowly with the molten metal and which will produce a vapor heavier than air.

In testimony whereof I affix my signature.

HAROLD H. OSBORNE.